

L. LA TOUR AND A. F. MUNNELL.

ROLLER FOR PRINTING PRESSES.

APPLICATION FILED MAY 29, 1919.

1,345,200.

Patented June 29, 1920.



Inventors

Lee LaTour  
and Anton F. Munnell,

By

Nairn A. Sturges.  
Attorney

# UNITED STATES PATENT OFFICE.

LEE LA TOUR AND ALTON F. MUNNELL, OF OMAHA, NEBRASKA, ASSIGNEES OF ONE-THIRD TO WARREN SMALL, OF OMAHA, NEBRASKA.

## ROLLER FOR PRINTING-PRESSES.

1,345,200.

Specification of Letters Patent. Patented June 29, 1920.

Application filed May 29, 1919. Serial No. 300,768.

To all whom it may concern:

Be it known that we, LEE LA TOUR and ALTON F. MUNNELL, citizens of the United States, residing at Omaha, in the county of Douglas and State of Nebraska, have invented certain new and useful Improvements in Rollers for Printing-Presses, of which the following is a specification.

This invention relates to an improvement in inking rollers, and has for one of its objects to provide inking rollers for printing presses which, while having an adequate degree of elasticity, will maintain its form regardless of changes in temperature, and especially will not become softened by operation of friction during continued use or long runs. Other objects include the provision of rollers which will be of lighter weight and more durable than ordinary, and will not become flattened or depressed from a circular form in cross-section when inadvertently left upon the ink-plate or other hard surface. The invention includes the use of certain ingredients to be mixed, calendered, and mounted upon a core or shaft and to be subjected to heat while in a mold.

The invention is fully described herein and in the appended claims and is illustrated in the accompanying drawing wherein,— Figure 1 is a side view of the inking roller and Fig. 2 is a view of the same in transverse section.

In making the inking rollers we have used the following ingredients:

|    |                             |         |
|----|-----------------------------|---------|
| 35 | Aluminum flake              | 2 lbs.  |
|    | Baryta                      | 2 lbs.  |
|    | Lime                        | ½ lb.   |
|    | Sulfur                      | 3½ lbs. |
| 40 | Magnesia                    | 4 lbs.  |
|    | Rubber, smoke-sheet, fine   | 34 lbs. |
|    | Rubber, smoke-sheet, coarse | 6 lbs.  |
|    | Degras                      | 2 oz.   |

The ingredients are mixed by any suitable means, and when thoroughly mixed the mass will have a consistency similar to that of bread dough, and the mass is then calendered or rolled into sheets of uniform thickness, the thickness not being important, but we have prepared the sheets with  $\frac{1}{2}$  of an inch in thickness in instances where the diameter of a roller was 2 inches.

The sheets are then applied to a shaft of

approximately one-half inch in diameter, said sheets being compactly rolled thereon to provide a required diameter of a roller, and after being placed in a mold is subjected, during a period of 40 minutes to a degree of heat within a scale from 270 to 290 degrees; and when removed from the mold the roller will present a smooth, finished appearance or surface.

In the accompanying drawing, numeral 3 indicates a shaft, upon which the sheets 4 are compactly mounted before being placed in a mold to be subjected to heat for producing the roller 5, and it will be understood that rollers of various diameters may be made, the sheets being mounted thereon as described; also it will be understood that the sheets may have a greater or lesser degree of thickness than mentioned, if desired.

While the proportions mentioned for the ingredients produce the best results and are preferred, certain changes, of course, are permissible. The amount of rubber may be reduced 20 per cent. if desired, the proportion of the other ingredients remaining the same; also milk or anilin oil may be substituted for the degras, as a softener, and baryta may be eliminated if desired, the other ingredients and their proportions remaining the same, and the proportions of the ingredients may be changed within a certain range, as expressed in the appended claims.

The advantages in the use of the ink roller as described will be appreciated since any melting or change in form from effects of heat will be eliminated, this being a matter of importance, another feature of importance being that any wearing away of the convexed surface from long usage or high degree of rotation will be practically avoided; also said surface will not become permanently flattened if allowed to lie upon an ink-plate or similar surface, and it is obvious that the comparatively light weight provided for these rollers is an advantage.

Having fully described our invention, what we claim and desire to secure by Letters Patent is,—

1. An inking roller, comprising a shaft, a sheet wound compactly upon the shaft and subjected to a vulcanizing heat, said sheet consisting of a part of the following in-

- 2
- 5 ingredients which include in weight, mixed aluminum flake, 2 lbs., baryta, 2 lbs., lime,  $\frac{1}{2}$  lb., sulfur,  $3\frac{1}{2}$  lbs., magnesia, 4 lbs., rubber smoke-sheet, fine,  $3\frac{1}{4}$  lbs., rubber smoke-sheet, coarse 6 lbs. and degras 2 oz.
- 10 2. An inking roller, comprising a shaft, a sheet wound upon the shaft and subjected to a heat approximately of 290 degrees, said sheet consisting of a part of the following ingredients which include approximately, in weight, aluminum flake, 2 lbs., lime,  $\frac{1}{2}$  lb., sulfur,  $3\frac{1}{2}$  lbs., magnesia, 4 lbs., rubber, 40 lbs., and a softening agent.
- 15 3. An inking roller comprising a shaft, a sheet wound upon the shaft and subjected to a vulcanizing heat, said sheet consisting of a part of the following mixed ingredients which include approximately, in weight, aluminum flake, 2 lbs., baryta, 2 lbs., lime,  $\frac{1}{2}$
- lb., sulfur,  $3\frac{1}{2}$  lbs., magnesia, 4 lbs., rubber, 20 40 lbs., and a softening agent.
4. An inking roller for printing presses, comprising a shaft, a cylindrical jacket circumscribing the shaft and subjected to a vulcanizing heat, the cylindrical jacket consisting of mixed ingredients in approximately the following proportions in weight, aluminum flake two parts, baryta two parts, lime one part, sulfur three parts, magnesia four parts, rubber forty parts, and degras 25 30 one-tenth part.

In testimony whereof, we have affixed our signatures in presence of two witnesses.

LEE LA TOUR.  
ALTON F. MUNNELL.

Witnesses:

ARTHUR H. STURGES,  
HIRAM A. STURGES.